

## UNITED STATES PATENT OFFICE

2,597,557

## NITRIC ACID TREATMENT OF POLYETHYLENE TEREPHTHALATE STRUCTURES

Leonard Edward Amborski, Buffalo, N. Y., assignor to E. I. du Pont de Nemours & Company, Wilmington, Del., a corporation of Delaware

No Drawing. Application May 25, 1949,  
Serial No. 95,379

3 Claims. (Cl. 8—115.5)

1

This invention relates to the manufacture of synthetic organic filaments, yarns, fibers, etc., and more particularly, to a novel process for treating filaments, yarns and like structures of polyethylene terephthalate whereby to improve certain physical properties thereof.

In many instances, e. g. where yarn is to be used as rug pile, etc., it is desirable to enhance the toughness, resilience, work recovery and allied physical properties of the filaments, fibers, or yarn. In general, filaments having a high degree of toughness, resilience, etc., also have high elongations at the breaking point, and it should therefore be possible to increase, say the toughness, of a given filament or yarn by increasing its elongation. However, expedients heretofore employed to improve elongation of filaments of synthetic organic materials, such as hot relaxing of a stretched filament, etc., for the most part work an improvement in elongation at the expense of the tenacity or tensile strength of the filament and often, while the desired degree of toughness is achieved, the tenacity of the resulting filaments are so low that the filaments are commercially inutile. These generalizations are particularly valid for filaments, fibers and yarns made from the synthetic linear polyethylene terephthalates disclosed in Whinfield and Dickson U. S. Patent No. 2,465,319 which filaments, fibers and yarns, because of their excellent physical and chemical properties, especially recommend themselves for broad application in the textile arts.

Obviously a treatment of such nature that satisfactory improvement in elongation, toughness, work recovery, etc., is obtained while retaining good tenacity, is to be highly desired. The improvement in these properties is attendant with a decrease in orientation of the polymer molecules along the fiber axis and an increase in the crystallinity of the polymer structures. Orientation along the fiber axis is achieved by submitting the fibers to the action of mechanical stress or stretching, either at the time of spinning or subsequent thereto, and results in improved tensile properties and pliability. This orientation is also evidenced by a characteristic X-ray diffraction diagram. In general, highly oriented yarn will exhibit relatively low elongation, resilience, work recovery and toughness.

An object of this invention therefore is to provide a simple, economical process for increasing the elongation of filaments, fibers, yarns and like funicular structures of polyethylene terephthalate without reducing the tenacity thereof to a detrimental level.

2

Another object is to produce tough filaments, fibers, yarns and like funicular structures of polyethylene terephthalate which have a desirably high tenacity at the breaking point.

5 A further object is to provide a simple, economical process for decreasing the orientation along the fiber axis of oriented filaments, fibers, yarns and like funicular structures of polyethylene terephthalate without reducing the tenacity thereof to a detrimental level.

10 A still further object is to render filaments, fibers, yarns and like structures of polyethylene terephthalate more crystalline and hence more stable.

15 These and other objects will more clearly appear hereinafter.

These objects are realized by the present invention which, briefly stated, comprises treating oriented filaments, fibers, yarns and like funicular structures of polyethylene terephthalate with nitric acid solution.

20 The polyethylene terephthalate structures with which this invention is concerned may be prepared by melt-spinning or casting the polymeric material by the usual techniques. The polymeric ethylene terephthalate may be prepared by the esterification of terephthalic acid with ethylene glycol under normal melt-polymerization conditions or again in a similar fashion by the ester exchange reaction between dimethyl terephthalate and ethylene glycol. The details of the preparation and shaping of polyethylene terephthalate are fully disclosed in the aforesaid patent to Whinfield and Dickson. Orientation along the fiber axis of the funicular structures is accomplished by a stretching operation, either integral with the spinning of the polyethylene terephthalate or at a subsequent time.

25 40 The concentration of the nitric acid solution may be varied within wide limits depending upon the extent of change of properties of the polyethylene terephthalate structures desired. For relatively short treatment times (from 10 seconds to 40 minutes) at room temperature, 50-80% nitric acid covers the most useful range. However, if shorter treatment times are desired, a higher concentration of acid and/or a higher temperature may be utilized if desired. Of course, it is to be understood that lower concentrations may be used if the increased length of time necessary to get the desired effect is unimportant.

30 45 50 55 With respect to the temperature conditions of the process of this invention, the range 0° C.—95° C. is the most useful. For ordinary purposes,

## 3

however, room temperature is preferred as being the most convenient operating temperature.

The treatment of this invention may be carried out on oriented filaments and yarns of polyethylene terephthalate under either relaxed conditions or under moderate tension, i. e. constant length. However, if treating tensions are too high, e. g., near the breaking point, an inferior product from the viewpoint of tenacity and elongation is produced.

The following examples of certain preferred embodiments further illustrate the principles and practice of this invention.

Inasmuch as this invention is concerned, in great part, with securing the maximum elongation while retaining good tenacity, the tenacity-at-break,  $T_0$ , calculated from the equation:

$$T_0 = T \left( 1 + \frac{E}{100} \right)$$

where  $T$  is the usual tenacity in grams per denier (g./d.) based on the measured denier (d.) and the measured break load (g.), and  $E$  is the measured percent elongation to break, serves as an excellent measure for comparing yarns and is used in the following examples to demonstrate the improvements herein realized.

## Example I

A 77-denier polyethylene terephthalate yarn that has been completely drawn with no subsequent relaxation is immersed in skein form in a 70% nitric acid solution at room temperature for a period of one minute. At the end of this time, it is withdrawn and immediately washed in a water bath. The following table shows the before and after properties and demonstrates clearly the large elongation increase at a useful level of tenacity.

| Treatment, Time | Tenacity, g./d. | Elongation | Denier | $T_0$ |
|-----------------|-----------------|------------|--------|-------|
| Control.....    | 6.55            | 12.3       | 77     | 7.35  |
| 1 Minute.....   | 2.97            | 95.0       | 132    | 5.8   |

The following example shows the effect of the nitric acid treatment on a polyethylene terephthalate funicular structure that has been drawn in two stages at two different temperatures without subsequent relaxation.

## Example II

The polyethylene terephthalate yarn for this example is drawn in two stages, first, it is drawn to 4 times its original length at 80° C. and, secondly, to 1.5 times its original length at 160° C. This yarn, which has a final denier of 61, is then immersed in a 70% nitric acid bath at room temperature for a period of time as indicated below with resulting physical properties as shown in the table. An untreated control is included for comparative purposes, together with a yarn highly relaxed by heat alone.

| Treatment, Time                    | Tenacity, g./d. | Elongation | Denier | $T_0$ |
|------------------------------------|-----------------|------------|--------|-------|
| Control.....                       | 7.38            | 11.3       | 61     | 8.35  |
| 10 Minutes.....                    | 4.4             | 62.3       | 85.3   | 7.12  |
| No Acid Treatment—Hot Relaxed..... | 2.8             | 62.0       | 80.0   | 4.53  |

The hot-relaxed sample above shows comparatively that for a high degree of relaxation, the acid treatment results in a far better yarn than

## 4

is possible by hot-relaxation alone. An acid-treated yarn having properties in this range is an extremely tough yarn (as indicated by the large area under its stress-strain curve) particularly useful for carpets.

## Example III

To show the usefulness of the process of this invention when applied to a partially relaxed yarn, a sample of the oriented yarn of Example II before treating was relaxed 10% and then given the same nitric acid treatment with the before and after results as shown below:

| Treatment, Time | Tenacity, g./d. | Elongation | Denier | $T_0$ |
|-----------------|-----------------|------------|--------|-------|
| Control.....    | 6.21            | 22.5       | 70     | 7.6   |
| 10 minutes..... | 5.17            | 44.3       | 82.7   | 7.46  |

The function of the nitric acid in the treatment of this invention seems to be that of a fiber penetrant which causes relaxation and does not appear to induce crosslinking or, for that matter, any irreversible effect. The following example shows that it is possible to redraw a nitric acid treated polyethylene terephthalate structure and get as a resultant product a funicular structure that has tenacity and elongation properties similar to the original starting material prior to nitric acid treatment. The following example illustrates the improvement in work recovery and initial tensile modulus over the control yarn for this particular modification of the treatment.

## Example IV

The oriented polyethylene terephthalate yarn is the same as that described in Example II. It is immersed in a 70% nitric acid bath for 10 minutes at room temperature, at which time, of course, it has the properties described for the treated yarn in Example II. It is then given a draw to 1.38 times its length at 205° C. and has the resultant properties as shown below. For comparative purposes the properties of the untreated control are also given.

| Properties                                 | Double-Drawn Control | Treated and Redrawn Yarn |
|--------------------------------------------|----------------------|--------------------------|
| Tenacity—g./d.....                         | 7.38                 | 7.2                      |
| Elongation—Per Cent.....                   | 11.3                 | 5.3                      |
| $T_0$ .....                                | 8.35                 | 7.6                      |
| Initial Tensile Modulus <sup>1</sup> ..... | 120.0                | 144.0                    |
| Work Recovery from <sup>2</sup> :          |                      |                          |
| 0.5% Elongation.....                       | 89.8                 | 100.0                    |
| 1.0% Elongation.....                       | 72.2                 | 84.0                     |
| 2.0% Elongation.....                       | 49.2                 | 58.0                     |

<sup>1</sup> Initial tensile modulus is defined as the slope of the first reasonably straight portion of a stress-strain curve of the yarn obtained by plotting tension as the vertical axis vs. elongation as the horizontal axis as the structure is being elongated at the rate of 10% per minute.

<sup>2</sup> Work recovery is defined as the ratio of the amount of work done by the yarn in recovering from deformation to the work recovery, a stress-strain curve, as described previously, is used under the following conditions: The yarn specimen is extended at a constant rate of elongation of 1% per minute; the specimen is held at the maximum elongation desired for 30 seconds and then is allowed to retract at the same rate at which it was extended. The same specimen is extended successively, 0.5, 1.0, and 2.0% for each determination. The areas under the elongation curve and the retraction curve respectively, represent work performed on the specimen, and work returned. These areas may be measured with a planimeter and the percent work recovery computed by means of the relation—

$$\text{Work recovery} = \frac{\text{area (work returned)}}{\text{area (work performed)}} \times 100$$

As an alternative use of the process of this invention, it is also possible to improve the work recovery of polyethylene terephthalate structures without appreciably affecting the tenacity, elon-

gation or initial tensile modulus. This is preferably done by treating the polyethylene terephthalate under constant length conditions, for example, on a stainless steel bobbin. The following example gives an illustration of this process and also shows the use of this invention at a temperature other than room temperature.

*Example V*

A polyethylene terephthalate yarn was double-drawn so that it had a final denier of 61 by drawing to 4 times its original length at 85° C., followed by a draw of 1.5 times its original length at 155° C. and had the properties as shown below as control. This yarn was then wound on stainless steel bobbin so that it was held taut at constant length. The yarn on the bobbin was then immersed in a 70% nitric acid solution for a period of 5 minutes at a temperature of 85° C. At the end of this time, it was withdrawn and washed and had the following physical properties:

| Properties                   | Control | Treated Yarn |
|------------------------------|---------|--------------|
| Tenacity—g./d.....           | 6.8     | 6.77         |
| Elongation—Per Cent.....     | 10.0    | 7.43         |
| Initial Tensile Modulus..... | 120.0   | 119.5        |
| Work Recovery from:          |         |              |
| 0.5% Elongation.....         | 89.9    | 95.1         |
| 1.0% Elongation.....         | 72.2    | 89.0         |
| 2.0% Elongation.....         | 49.2    | 71.0         |

Additionally, the process of this invention operates to give a resultant structure that, on X-ray analysis, proves to be considerably more crystalline than the untreated control. This is probably due to the fact that nitric acid as a fiber penetrant allows the crystallites in the structure greater freedom of movement. The increased crystallinity is a useful result inasmuch as it represents a more stable configuration. That such an increase does occur is clearly shown by the conventional X-ray diffraction diagrams. Such diagrams show e. g., that the spots in the diagram obtained from crystalline double-drawn polyethylene terephthalate are made narrower by nitric acid relaxation, indicating increased crystallization. At the same time the spots are narrowed, they are lengthened into arcs, which phenomenon corresponds to decreased orientation.

Although the invention has been described herein above with specific reference to funicular structures such as filaments, fibers and yarns it is obvious that the novel effects and advantages thereof will pertain as well to other structures

such as film, ribbons, rods, etc., of polyethylene terephthalate.

The invention provides an inexpensive method of relaxing large quantities of yarn in a short time, and yield in an economical and simple fashion an extremely tough yarn, which has a relatively high tenacity, an improved work recovery, a high initial tensile modulus, and a high degree of crystallinity.

10 As many apparent and widely different embodiments can be made without departing from the spirit and scope of this invention it is to be understood that said invention is in no wise restricted except as set forth in the appended claims.

I claim:

1. A method for improving the elongation characteristics of drawn, oriented yarns, filaments, and fibers of polyethylene terephthalate 20 which comprises contacting said structures with an aqueous nitric acid solution at a temperature of from 0° C. to 95° C. until structures of the desired elongation and tenacity are obtained and thereafter washing said structures and drying 25 same, whereby to produce drawn structures having increased elongation.

2. A method for improving the elongation characteristics of drawn, oriented yarns, filaments, and fibers of polyethylene terephthalate 30 which comprises relaxing said structures in an aqueous nitric acid solution at a temperature of from 0° C. to 95° C. until structures of the desired elongation and tenacity are obtained and thereafter washing said structures and drying same, 35 whereby to produce drawn structures having increased elongation.

3. A method for improving the elongation characteristics of drawn, oriented yarns, filaments, and fibers of polyethylene terephthalate 40 which comprises relaxing said structures in a 50-80% nitric acid solution for 10 seconds to 40 minutes at room temperature.

LEONARD EDWARD AMBORSKI.

REFERENCES CITED

45 The following references are of record in the file of this patent:

UNITED STATES PATENTS

50 Number Name Date  
2,465,319 Whinfield et al. ---- Mar. 22, 1949

FOREIGN PATENTS

55 Number Country Date  
610,135 Great Britain ---- Oct. 12, 1948